# EUROPEAN PATENT SPECIFICATION

(11) **EP 0 049 706 B1**
(45) Date of publication and mention of the grant of the patent: **01.04.1987**
(21) Application number: 80106171.4
(22) Date of filing: 10.10.1980
(51) Int. Cl.: C23C 22/10, C23C 22/50

(54) **Method and apparatus for continuously forming color display layer on stainless steel strip**
Verfahren und Apparat zur kontinuierlichen Bildung einer farbigen Dekorschicht auf einem rostfreien Stahlband
Procédé et appareil pour la fabrication en continu d'une pellicule décorative colorée sur un ruban d'acier inoxydable

(43) Date of publication of application: 21.04.1982
(73) Proprietor: NIPPON KINZOKU CO., LTD., Tokyo (JP)
(72) Inventor: Yoshihara, Tsuyoshi, Sanjo-shie Niigata-ken (JP); Ohashi, Nobuaki, Niiza-shi Saitama-ken (JP)
(74) Representative: Klöpsch, Gerald, Dr.-Ing. Patentanwalt

## Description

This invention relates to a method for continuously forming a color display layer on the surface of stainless steel.

A color display layer (or oxide layer) formed on the surface of stainless steel exhibits a metallic luster of various color tones and, thus produces a highly decorative effect. Techniques of forming such a color display layer are disclosed in, for example, British Patent Specifications 1,122,172 and 1,122,173. In any of the prior arts exemplified above, stainless steel, having the surface sufficiently polished in advance, is immersed in a mixture of sulfuric acid and chromic acid so as to form a color display layer on the surface of the stainless steel, followed by subjecting the color display layer to a hardening treatment by electrolysis in a mixture of phosphoric acid and chromic acid. It should be noted that the resultant color display layer is markedly influenced by the composition and temperature of the oxidizing liquor, i.e., acid mixture, as well as by the surface conditions of the stainless steel, rendering it absolutely necessary to control accurately the oxidizing solution and stainless steel for obtaining a color display layer of a desired color tone.

In order to control the color tone of the color display layer, it is proposed to monitor the potential difference between the stainless steel immersed in the oxidizing solution and a reference electrode, in view of the fact that the potential difference mentioned, changes with time in accordance with growth in the thickness of the color display layer. This control method is certainly effective where a color display layer is formed on a stainless steel plate on a batch system. But, where a stainless steel strip is continuously immersed in an oxidizing solution, it is impossible to utilize changes which occur with time in potential difference between the reference electrode and the strip immersed in the oxidizing solution because the potential difference mentioned is maintained substantially constant. It should also be noted that the color tone of the color display layer is remarkably influenced by the material and surface condition of stainless steel and the composition and temperature of the oxidizing solution even if the potential difference in question is maintained constant. It follows that the color tone of the color display layer formed in one case is not necessarily equal to that of the color display layer formed in another case. Under the circumstances, it was customary to control the immersion time of a stainless steel strip in an oxidizing solution based mainly on experiences where a color display layer of a desired color tone is continuously formed on the strip, leading to nonuniformity in color tone of the color display layers.

GB-A-1 518 296 discloses a method of forming a color display layer on surface of a stainless steel sheet by immersing the sheet in an oxidizing solution, comprising the steps of
- immersing a standard sample of the steel in an oxidizing solution for forming a color display on the surface of the sample, thereby establishing a relationship between the thickness or color tone of the color display layers and the potential difference between the sample immersed in the oxidizing solution and a reference electrode
- immersing the same kind of stainless steel sheet in said oxidizing solution for forming a color display layer on the surface of the sheet, the difference in thickness between the actually formed color display layer and a desired color display layer being converted to a difference in potential difference on the basis of the relationship measured first and the immersion time of sheet in the oxidizing solution being controlled on the basis of said difference in potential difference. The method is not carried out continuously.

Further it was also customary to employ a batch system in which the color display layer formation and the hardening treatment of the color display layer are carried out independently, with the result that it was difficult to obtain stainless steel strips bearing color display layers on uniform color tone. For overcoming the difficulty mentioned, it is thought effective to pass a long stainless steel strip continuously through an oxidizing solution for forming a color display, i.e., oxide film on the strip and through an electrolytic solution for hardening the color display layer. In the conventional continuous treatment, however, part of the current for the electrolytic solution tends to flow into the oxidizing solution through the stainless strip under treatment, rendering it difficult to measure the natural potential of the strip and, thus, to control-the thickness of the oxide film. In other words, it is absolutely necessary to solve the above-noted problem for bringing a continuous treatment into practical uses.

One object of this invention is to provide a method of continuously formirrg a color display layer on the surface of a stainless steel strip by immersing the strip in an oxidizing solution, in which the potential difference between the strip immersed in the oxidizing solution and a reference electrode is utilized for controlling the immersion time of the strip in the solution.

According to this invention, there is provided a method of forming a color display layer on the surface of a stainless steel strip by immersing the strip in an oxidizing solution which comprises the steps of
(a) immersing a stainless steel strip (A) in an oxidizing solution in a tank in order to form a color display layer on the surface of the strip (A) which is electrically insulated from the tank, thereby allowing the generation of an electrical potential difference between the strip and the tank and establishing the relationship between the color tone or the thickness of the color display layer and the potential difference between the strip (A) being immersed in the oxidizing solution and either a reference electrode (5) or the immersion time,
(b) immersing a particular stainless steel strip (A) of the same kind in said oxidizing solution in order to form a color display layer on the surface of said strip (A),

characterised by the steps of comparing the obtained color display layer with a desired color display layer, determining the difference in potential difference versus the reference electrode between the obtained color display layer and the desired one on the basis of the relationship established in step (a) and adjusting the immersion time in order to obtain the potential difference between the strip and the reference electrode corresponding to the desired color display layer and further characterized in that the stainless steel strip is treated continuously.

Additional features of the invention are set forth in the attached dependant claims.

The invention method for continuously forming a color display layer on the surface of a stainless steel strip by immersing the strip in an oxidizing solution in a tank can be carried out in an apparatus comprising:
a means for measuring the potential difference between the strip and a reference electrode immersed in the oxidizing solution: a means for measuring the color (or thickness) of the color display layer; a means for controlling the immersion time on the basis of a relationship between the thickness of the color display layer and said potential difference; a means for rinsing the color display layer; a tank containing a hardening solution, and a means for conducting an electrical current between the strip and an electrode immersed in the hardening solution, wherein the connections in the electrical circuits for respectively measuring the potential difference and applying an electrolysis current are separated and an electric current is not formed between the strip and the reference electrode immersed in the oxidizing solution so as to generate a potential difference therebetween.

This invention can be more fully understood from the following detailed description when taken in conjunction with the accompanying drawings, in which:
-Fig. 1 is a schematic cross sectional view showing an apparatus used for continuously forming a color display layer on the surface of a stainless steel strip according to the method of this invention.
Fig. 2 is a graph showing the relationship between the thickness (or color tone) of a color display layer and the potential difference between the stainless steel band immersed in an oxidizing solution and a reference electrode.
Fig. 3 is a schematic cross sectional view showing an apparatus for carrying out the inventive method.
Fig. 4 to 6 are schematic cross sectional views each showing a conventional apparatus for comparison with this invention.

Before forming a color display layer, the surface of a stainless steel strip is polished by, for example, buffing or chemical polishing. In this step, the surface of the strip may be patterned by etching or embossing. The surface polishing should be carried out thoroughly because uneven polishing causes unevenness in the color tone of the formed color display layer. After the surface polish, the stainless steel strip should be cleaned and water-washed so as to remove completely the oil and fat as well as dust from the strip. For the cleaning, it is possible to employ ordinary methods such as immersion in an alkaline solution and electrolysis.

After completion of the pretreatment, a stainless steel strip A is passed successively through an oxidizing solution tank 1, a water tank 2, a hardening solution tank 3 and a water tank 4 as shown in Fig. 1. An oxide film, i.e., color display layer, is formed on the surface of the strip A within the tank 1 and, after water-washed within the tank 2, hardened within the tank 3 by means of electrolysis. Finally, the strip A bearing the hardened color display layer is washed with water within the tank 4 and rolled up. In this fashion, a color display layer is formed continuously on the surface of the strip A.

A mixture of sulfuric acid and chromic'acid, or bichromate is used as the oxidizing solution. In order to form a uniform oxide film on the surface of the strip A in a short time, the mixture should generally consist of 450 to 800 g/l of sulfuric acid and 50 to 350 g/l of chromic acid. Desirably, the mixture should be kept at 70 to 120°C. The thickness of the oxide film is controlled on the basis of the natural potential of the stainless steel strip A. Specifically, a reference electrode 5 formed of, for example, platinum is immersed in the oxidizing solution in a manner to face the strip A. Further, the reference electrode 5 and the strip A are connected to a potentiometer 7 via lead wires 6 so as to form a circuit 8 for measuring the potential difference between the electrode 5 and the strip A. Naturally, the oxide film thickness is controlled on the basis of the indication of the potentiometer 7. In general, the strip A is immersed in the oxidizing solution for about 10 minutes, though the immersion time depends on the desired color of the color display layer as well as on the temperature and composition of the oxidizing solution containing chromic acid or potassium bichromate. It should be noted that the oxidizing solution tank 1 is disposed on a substrate 10 with an insulating member 9 such as rubber interposed therebetween so as to electrically insulate the strip A from the tank 1. Otherwise, an electric circuit is formed between the strip A and the tank 1, with the result that the strip A and the tank 1 are allowed to bear the same potential. In this case, it is of course impossible to form an oxide film on the surface of the strip A. The material of the tank 1 is not particularly restricted, though a metal nobler than the stainless steel strip A may be used for forming the tank 1.

The immersion time of strip A in the liquor is controlled on the basis of the potential difference between strip A and a reference electrode 5 formed of, for example, platinum and immersed in solution. To be more specific, the relationship between the potential difference mentioned above and the thickness or color tone of the color display layer formed on the stainless steel strip is measured first by continuously immersing the strip in the solution. Lines a, b, c shown in Fig. 2 represent the relationship mentioned above. It should be noted that the same potential difference does not necessarily bring about the same thickness of the color display layer as seen from Fig. 2. This is because subtle influences are given to the process of forming the color display layer by the material and surface condition of the stainless steel strip as well as by the composition of the oxidizing solution. It should also be noted, however, that the graphs of the color display layer thickness relative to the potential difference are inclined at almost the same angle. In other words, the difference in potential difference between two optional color tones of the color display layer is constant. For example, the difference between blue and green is 3.2 mV and the difference between blue and grey is 0.5 mV. The reason for this phenomenon is unclear.

After preparation of a graph as shown in Fig. 2, the stainless steel strip A is continuously immersed in the oxidizing solution contained in the tank 1 so as to form a color display layer on the surface of the strip A. In this step, the immersion time of the strip in the solution is set optionally. Potential difference between the reference electrode 5 and strip A during the operation is measured together with the thickness or color tone of the formed color display layer. Then, difference in potential difference between the color tone of the color display layer and a desired color tone is determined based on the graph of Fig. 2 so as to control the immersion time of strip A in a manner to form a color display layer of the desired color tone. Suppose the color display layer actually formed is grey and it is desired to form a blue color display layer. In this case, the difference in potential difference is 0.5 mV as seen from Fig. 2. Thus, the immersion time is shortened such that the potential difference between the reference electrode 3 and strip A is made 0.5 mV smaller than the initially measured value. Where it is intended to form a golden color display layer, the immersion time is prolonged such that the potential difference mentioned is made larger than the initially measured value by 0.6 mV (difference between gold and grey is 0.6 mV). After the desired color tone has been obtained, the stainless steel strip is continuously passed through the oxidizing solution at a constant potential.

It is possible to control manually, the immersion time, or running speed, of the stainless steel strip. Alternatively, the immersion time can be controlled automatically. In this case, the difference in potential difference is automatically detected and the detected signal is supplied to the driving means of the stainless steel strip so as to control the immersion time of the strip in the oxidizing solution.

The stainless steel strip A having an oxide film formed thereon is washed with water within the water tank 2 and, then, immersed in the hardening solution contained in the tank 3. The oxide film is hardened within the hardening solution by means of electrolysis. Specifically, a mixture of phosphoric acid and chromic acid, which is used as the hardening solution, is electrolyzed so as to allow the metal chromium atoms or chromium hydroxide liberated by the electrolysis to bill the pores of the oxide film and, thus, to harden the oxide film. As shown in Fig. 1 a current conducting means 14 utilized in the electrolysis comprises an anode 11 formed of, for example, lead, which is immersed in the hardening solution, the strip A acting as a cathode, and a DC power source 13 connected between the anode and cathode via lead wires 12. In general, the electrolysis is performed for about 10 minutes under a current density of 0.2 to 0.3 A/ dₘ₂.

It is important to note that the stainless steel strip A included in the circuit 8 for measuring the natural potential of the strip A is separated from the current conducting means 14. In other words, the circuit 8 and the current conducting means 14 are separate from each other. It follows that the current flowing through the electrolytic system scarcely flows into the circuit 8, with the result that the indication of the potentiometer 7 is stabilized and, thus, the thickness of the oxide film formed on the strip A can be controlled without difficulty. Incidentally, the strip A is guided by guide rollers 15. Further, both the strip A and the substrate 10 are connected to the ground via lead wires 16 and 17.

Fig. 3 shows an apparatus for carrying out the inventive method. The embodiment of Fig. 3 differs from the embodiment of Fig. 1 in the connection points of the stainless steel strip A to the circuit 8 and to the current conducting means 14, though the strip A included in the circuit 8 is electrically separated from the current conducting 14 in Fig. 3 as in Fig. 1. To be brief, it is possible to modify the embodiment of Fig. 1 as far as the circuit 8 for measuring the natural potential of the strip A is separate from the electrolytic system.

The stainless steel which can be treated by the method of this invention includes, for example, austenite series stainless steel such as SUS 301, 302, 304, 316, 321 and ferrite series stainless steel such as SUS 405, 430, 434.

### Example 1

A stainless steel strip was actually treated by the method of this invention. Specifically, a stainless steel strip of SUS 304 with a polished surface, was degreased and then passed through an oxidizing liquor maintained at 89°C and consisting of 540 g/l of sulfuric acid and 240 g/l of chromic acid at a speed of 70 cm/min. Since the effective length of the tank containing the solution was 3,500 mm, the immersion time of the strip in the solution was 5.0 minutes. A grey color display layer was formed on the surface of the strip. Further, the potential difference between the reference electrode and the stainless steel strip was found to be -191.6 mV. Then, the potential difference mentioned was set as 192.3 mV, which is lower by 0.7 mV than the initial value, by increasing the strip running speed to 82 cm/min so as to form a desired blue color display layer. Incidentally, difference in potential difference between grey and blue 0.7 mV. Thereafter, the strip running speed was controlled so as to maintain the potential difference at -192.3 mV. The resultant stainless steel strip had a color display layer of uniform color tone.

### Example 2

Stainless steel strips were continuously treated by using an apparatus as shown in Fig. 1. A mixture of 295 g/I of chromic acid and 502 g/l of sulfuric acid, which was maintained at 85°C, was used as the oxidizing solution. Also, a mixture of 250 g/l chromic acid and 2.5 g/l of phosphoric acid was used as the hardening solution and electrolysis was carried out under a current density of 0.3 A/dm². Further, the immersion time of the strip in the hardening solution was 10 minutes.

The running speed of one of the stainless steel strips through the oxidizing solution was controlled in a manner of form a blue color display layer on the surface of said strip. Specifically, the running speed mentioned was controlled in a manner to allow the potentiometer 8 to indicate -185.0 to -185.3 mV. The treatment was continued for about 4 hours, with the result that the entire surface of the strip was covered with a blue color display layer.

In order to form a golden color display layer on the surface of the strip, the running speed in question was controlled in another treatment in a manner to allow the potentiometer to indicate -184.4 to -184.7 mV. The treatment was continued for about 4 hours, with the result that the entire surface of the strip was covered with a golden color display layer.

In still another treatment, it was intended to form a green color display layer. To this end, the running speed of the strip through the oxidizing solution was controlled in a manner to allow the potentiometer to indicate -182.4 to -182.7 mV. The treatment was continued for about 4 hours, with the result that the entire surface of the strip was covered with a green color display layer.

Further, the color tone of the golden color display layer formed on the stainless steel strip was measured at an interval of 2.5 m over a strip length of 350 m, and Hunter's formula was applied to the color tones thus measured for determining a color difference AE, with the result that the standard deviation a of AE was 1.01.

### Control 1

Stainless steel strips were continuously treated as in Example 2 except that the potentiometer 8 was removed from the treating apparatus.

In one of the operations, the running speed of the strip through the oxidizing solution was set in advance in a manner to form a blue color display layer on the surface of the strip. The treatment was continued for 4 hours, maintaining constant the strip running speed mentioned above. The color display layer formed in the late stage of the treatment was found to be somewhat reddish. The change in composition of the oxidizing solution caused by evaporation, etc. is thought to have brought about the color change of the color display layer.

In another operation, the strip running speed was set in a manner to form a golden color display layer on the strip and the treatment was continued for 4 hours, maintaining constant the strip running speed. As in Example 2, a color difference AE of the resultant color display layer was determined by Hunter's formula. The standard deviation 5 was found to be as large as 1.83 in contrast to 1.01 for Example 2. This substantiates that the control of the potential difference between the stainless steel strip and the reference electrode immersed in the oxidizing solution is very important for forming a color display layer of uniform color tone.

### Control 2

Stainless steel strips were treated as in Example 2 except that the oxidizing solution tank 1 was directly connected electrically to the ground. Naturally, an electric circuit was formed between the tank 1 and the strip. In this case, a color display layer was not formed at all on the surface of the treated strip.

An additional treatment was conducted as in Example 2 except that an apparatus as shown in Fig. 3 was used in place of the apparatus shown in Fig. 1. In this case, however, the oxidizing solution tank 1 was directly disposed on the substrate 10; namely, the insulating member 9 disposed between the tank 1 and the substrate 10 was removed in this experiment. A color display layer was not formed at all on the surface of the treated stainless steel strip.

### Control 3

An apparatus as shown in Fig. 4 was used for continuously treating a stainless steel strip. It is important to note that, in the apparatus of Fig. 4, the strip included in the potential difference- measuring circuit 8 is also included in the current conducting means 14.

During the treatment, the indication of the potentiometer 7 was greatly vibrated over a range of several milli-volts because of the influence given by the current flowing in the electrolytic system, making it difficult to control the electric potential, with the result that the color display layer formed on the surface of the strip was quite non-uniform in color tone.

Likewise, an apparatus as shown in Fig. 5 was used for continuously treating a stainless steel strip. In this case, it was impossible to recognize the indication of the potentiometer 7 because of the influence given by the current flowing in the electrolytic system. Of course, it was substantially impossible to control the color tone of the color display layer formed on the strip.

Further, an apparatus as shown in Fig. 6 was used for continuously treating a stainless steel strip. As apparent from the drawing, the take-up roll as well as the feed roll was electrically connected to the ground in the apparatus used. In this case, the indication of the potentiometer 7 was vibrated over a range of several milli-volts because of the influence of the current flowing in the electrolytic system, with the result that the color display layer formed on the surface of the strip was quite non-uniform.

It is important to note that, in the present invention, the stainless steel strip included in the circuit for measuring the natural potential is electrically separated from the current conducting means. Thus, the natural potential-measuring circuit is not influenced by the current conducting means, with the result that the thickness of the oxide film formed on the surface of the strip can be controlled stably. It follows that the method and apparatus of this invention permit continuously treating a long stainless steel strip so as to form a color display layer of a uniform color tone on the entire surface of the strip.

As described above in detail, this invention is based on the finding that the thickness (or color tone) of a color display layer is strongly related to the potential difference between the stainless steel strip immersed in the oxidizing solution and the reference electrode in the process of continuously forming a color display layer on the surface of a stainless steel strip. Specifically, the particular relationship between the thickness and the potential difference mentioned above is utilized for controlling the immersion time of the stainless steel strip in the oxidizing solution. This renders it possible to control the immersion time accurately and to form a color display layer of uniform color tone. In addition, the immersion time can be controlled automatically.

In the process described above, a mixture of sulfuric acid and chromic acid is used as the oxidizing solution. However, it is possible to use a different oxidizing solution in the method of this invention.

## Claims

1. Method of forming a color display layer on the surface of a stainless steel strip by immersing the strip in an oxidizing solution which comprises the steps of:
(a) immersing a stainless steel strip (A) in an oxidizing solution in a tank in order to form a color display layer on the surface of the strip (A) which is electrically insulated from the tank, thereby allowing the generation of an electrical potential difference between the strip and the tank and establishing the relationship between the color tone or the thickness of the color display layer and either the potential difference between the strip (A) being immersed in the oxidizing solution and a reference electrode (5) or the immersion time,
(b) immersing a particular stainless steel strip (A) of the same kind in said oxidizing solution in order to form a color display layer on the surface of said strip (A),
characterised by the steps of comparing the obtained color display layer with a desired color display layer, determining the difference in potential difference versus the reference electrode between the obtained color display layer and the desired one on the basis of the relationship established in step (a) and adjusting the immersion time in order to obtain the potential difference between the strip and the reference electrode corresponding to the desired color display layer and further characterised in that the stainless steel strip is treated continuously.

2. The method according to claim 1, wherein the oxidizing solution consists of 450 to 800 g/l of sulfuric acid and 50 to 350 g/l of chromic acid or bichromate.

3. The method according to claim 2, wherein the oxidizing solution is maintained at 70 to 120°C.

4. The method according to any one of claims 1 to 3, wherein either one of the stainless steel strip (A) and a tank (1) containing the oxidizing solution is insulated from the ground.

5. The method according to claim 1, wherein the stainless steel strip is further introduced into a hardening solution after being rinsed, and a power source is provided between the strip and an electrode immersed in the hardening solution thereby providing an electrical circuit which is electrically separated from an electrical circuit in the oxidizing solution for measuring the potential difference.

## Patentansprüche

1. Verfahren zur Bildung einer farbigen Dekorschicht auf einem rostfreien Stahlband durch Eintauchen des Stahlbandes in eine oxidierende Lösung mit den folgenden Schritten:
(a) Eintauchen eines rostfreien Stahlbandes (A) in eine sich in einem Tank befindliche, oxidierende Lösung, um eine farbige Dekorschicht auf der Oberfläche des Bandes (A) zu bilden, welches elektrisch isoliert vom Tank ist, wobei eine elektrische Spannung zwischen dem Band und dem Tank erzeugt wird und eine Relation zwischen dem Farbton oder der Dicke der farbigen Dekorschicht und entweder der elektrischen Spannung des Bandes (A), das in die oxidierende Lösung getaucht wurde, und einer Referenzelektrode (5) oder der Eintauchzeit herstellt wird
(b) Eintauchen eines bestimmten rostfreien Stahlbandes (A) von gleicher Beschaffenheit in die oxidierende Lösung, um eine farbige Dekorschicht auf der Oberfläche des Bandes (A) zu bilden,
dadurch gekennzeichnet, daß die erhaltene farbige Dekorschicht mit der gewünschten farbigen Dekorschicht verglichen wird und der Unterschied der elektrischen Spannung gegenüber der Referenzelektrode zwischen der erhaltenen und der gewünschten farbigen Dekorschicht festgelegt wird aufgrund der Relation, die in Schritt (a) bestimmt wurde, und die Eintauchzeit angepaßt wird, um die elektrische Spannung zwischen Band und Referenzelektrode entsprechend der gewünschten farbigen Dekorschicht zu erhalten, und daß das rostfreie Stahlband ununterbrochen behandelt wird.

2. Verfahren nach Anspruch 1, dadurch gekennzeichnet, daß die oxidierende Lösung aus 450 bis 800 g/l Schwefelsäure und 50 bis 350 g/l Chromsäure oder Dichromat besteht.

3. Verfahren nach Anspruch 2, dadurch gekennzeichnet, daß die oxidierende Lösung bei Temperaturen zwischen 70 und 120°C gehalten wird.

4. Verfahren nach einem der Ansprüche 1 bis 3, dadurch gekennzeichnet, daß sowohl das rostfreie Stahlband (A) als auch der Tank mit der oxidierenden Lösung vom Boden isoliert sind.

5. Verfahren nach Anspruch 1, dadurch gekennzeichnet, daß das rostfreie Stahlband nach einer Spülung in eine härtende Lösung gebracht wird, und eine Energiequelle zwischen Band und einer Elektrode, die in die härtende Lösung getaucht wurde, angebracht wird, wodurch ein elektrischer Kreislauf entsteht, der elektrisch isoliert ist von einem elektrischen Kreislauf in der oxidierenden Lösung zur Messung der Spannung.

## Revendications

1. Procédé pour former une pellicule d'aspect coloré à la surface d'un ruban d'acier inoxydable en immergeant le ruban dans une solution oxydante, comportant les étapes de:
a) immerger un ruban d'acier inoxydable (A) dans une solution oxydante qui se trouve dans une cuve pour former une pellicule d'aspect coloré à la surface du ruban (A) qui est électriquement isolé d'avec la cuve, autorisant ainsi l'apparition d'une différence de potentiel électrique entre le ruban et la cuve et établissant la relation entre la tonalité de la couleur ou l'épaisseur de la pellicule d'aspect coloré et soit la différence de potentiel entre le ruban (A) immergé dans la solution oxydante et une électrode de référence (5), soit la durée d'immersion.
b) immerger un ruban particulier d'acier inoxydable (A) de même type dans ladite solution oxydante pour former une pellicule d'aspect coloré à la surface dudit ruban (A),
caractérisé par les étapes consistant à comparer la pellicule d'aspect coloré obtenu avec la pellicule d'aspect coloré désiré, à déterminer l'écart de différence de potentiel, par rapport à l'électrode de référence, entre la pellicule d'aspect coloré obtenu et celui désiré sur la base de la relation établie dans l'étape (a) et ajuster la durée d'immersion pour obtenir entre le ruban et l'électrode de référence la différence de potentiel correspondant à la pellicule d'aspect coloré désiré; et caractérisé en outre en ce que le ruban d'acier inoxydable est traité en continu.

2. Procédé selon la revendication 1, dans lequel la solution oxydante est constituée de 450 à 800 g/ 1 d'acide sulfurique et de 50 à 350 g/l d'acide chromique ou bichromate.

3. Procédé selon la revendication 2, dans lequel la, solution oxydante est maintenue à une température de 70 à 120°C.

4. Procédé selon l'une quelconque des revendications 1 à 3, dans lequel on isole du sol soit le ruban d'acier inoxydable (A) soit une cuve (1) contenant la solution oxydante.

5. Procédé selon la revendication 1, dans lequel on introduit en outre le ruban en acier inoxydable dans une solution durcissante après l'avoir rincé et dans lequel on prévoit une source d'énergie électrique entre le ruban et une électrode immergée dans la solution durcissante, réalisant ainsi un circuit électrique qui est électriquement isolé du circuit électrique qui passe dans la solution oxydante pour mesurer la différence de potentiel.
